

June 5, 1973

G. L. TURNER ET AL

3,737,505

PROCESS FOR MANUFACTURE OF HIGH SHEEN BIFILAMENT  
YARN AND ELASTIC TEXTILE ARTICLE

Filed May 28, 1971

4 Sheets-Sheet 1



FIG. 1

FIG. 1A



FIG. 2



FIG. 3

INVENTORS  
RALPH W. SCHUETTLEF  
GARLAND L. TURNER  
GEORGE H. COLLINGWOOD

BY

*Roy H. Messingill*  
ATTORNEY

June 5, 1973

G. L. TURNER ET AL  
PROCESS FOR MANUFACTURE OF HIGH SHEEN BIFILAMENT  
YARN AND ELASTIC TEXTILE ARTICLE

3,737,505

Filed May 28, 1971

4 Sheets-Sheet 2

FIG.4



FIG.5



FIG.6



FIG.7



INVENTOR.  
RALPH W. SCHUETTLER  
GARLAND L. TURNER  
GEORGE H. COLLINGWOOD

BY

*Roy W. Massengill*  
ATTORNEY

June 5, 1973

G. L. TURNER ET AL  
PROCESS FOR MANUFACTURE OF HIGH SHEEN BIFILAMENT  
YARN AND ELASTIC TEXTILE ARTICLE

3,737,505

Filed May 28, 1971

4 Sheets-Sheet 3

FIG.8



FIG.9



FIG.10



FIG.11



FIG.12



FIG.13



INVENTORS

RALPH W. SCHUETTLER  
GARLAND L. TURNER  
GEORGE H. COLLINGWOOD

BY

*Roy H. Massengill*

ATTORNEY

June 5, 1973

G. L. TURNER ET AL  
PROCESS FOR MANUFACTURE OF HIGH SHEEN BIFILAMENT  
YARN AND ELASTIC TEXTILE ARTICLE

3,737,505

Filed May 28, 1971

4 Sheets-Sheet 4



FIG. 14



FIG. 15



FIG. 16

F.T. = FALSE TWIST



FIG. 17



FIG. 18



FIG. 19

F.T. = FALSE TWIST

INVENTORS  
RALPH W. SCHUETTLER  
GARLAND L. TURNER  
GEORGE H. COLLINGWOOD

BY

*Key H. Messing, III*  
ATTORNEY

3,737,505

## PROCESS FOR MANUFACTURE OF HIGH SHEEN BIFILAMENT YARN AND ELASTIC TEXTILE ARTICLE

Garland Linwood Turner, Chesterfield, Va., Ralph William Schuettler, Fuguey Varina, N.C., and George Howard Collingwood, West Warwick, R.I., assignors to Allied Chemical Corporation, New York, N.Y.

Continuation-in-part of applications Ser. No. 733,556 and Ser. No. 733,557, both May 31, 1968. This application May 28, 1971, Ser. No. 148,125

Int. Cl. B28h 21/54

U.S. CL. 264—177 F

3 Claims

### ABSTRACT OF THE DISCLOSURE

A bifilament yarn comprising two symmetrical lobes fused so that the concave sides intercept at angle  $\theta$  ranging from 10 to 54°. The yarn has a broad concave area and a narrow edge area of convex shape and preferably a modification ratio of between 1.65 and 3.0. This bifilament yarn, textured and non-textured, semidull and bright, when converted to plain knit hosiery has a luster in the range of 6.6 to 21 ( $K/S \times 100$ ) units. The textured and non-textured plain knit textile articles consisting of the bifilament yarns of this invention after repetitive elongations of 25 percent have 150–300 percent greater work of recovery and equal improvement in resistance to sagging and wrinkling than other cross-sectional configurations. The bifilament yarns are prepared by melt spinning thermoplastic homopolymers having a relative formic acid viscosity of 25 to 90 at a temperature of 250–280° C. through twin orifices separated from each other for a distance of 0.05 to 4.0 mils.

### BACKGROUND OF THE INVENTION

This is a continuation-in-part application of Ser. Nos. 733,556 and 733,557, filed May 31, 1968, now abandoned.

Ladies' stretch hosiery has usually been made from false-twisted round cross section yarn or bicomponent yarn where one component is a homopolymer and the other component is a copolymer arranged either side by side with the homopolymer or as a core in a sheath and core arrangement. Such yarns, while finding utility in ladies' hosiery, have a disadvantage in that three or more sizes are required to cover the range of sizes 8½ to 11½. This range of sizes amounts to about 99 percent of the ladies' hosiery consumption in the United States. Additionally, various cross-sectional types such as trifilament, triangular, Y-cross section, star cross section, polygonal, and the like, have been employed to achieve decorative effects in these hosiery. When these conventional yarns are employed, three or more sizes are required to cover the practical range of hosiery sizes, and generally, the modified hosiery has either too dull an appearance or too much glitter with the latter having utility only for its novelty effect.

There has long been a need for a true stretch hosiery where one size will fill the majority of end-use requirements and which has sufficient luster and sheen to be desirable for formal wear without being too gaish for everyday and business use. It is also highly desirable to produce a true stretch yarn having adequate power of recovery to maintain a good fit without wrinkling or becoming permanently deformed under severe bending action, such as deep-knee bends. Additionally, hosiery yarns made from two components, a homopolymer and a copolymer, are expensive and difficult to produce. Thus,

there has long been a need to produce a stretch yarn which avoids the described problems, and more particularly, it has been desirable to produce said yarn from a single homopolymer.

5 In an attempt to simulate some of the geometric forms of natural fibers, various configurations including bifilament yarns were produced almost four decades ago from man-made cellulosic fibers as disclosed in Swiss Pat. 145,408 dated Feb. 28, 1931. Since this time, several 10 patents have been issued showing various configurations representing a range of fiber types which have two or more lobes. For example, U.S. Pats. 3,156,607 and 3,131-427 illustrate yarn configurations which are essentially bilobal. Thus, the prior art is replete with patents showing 15 various types of bilobal yarns yet none of the patentees recognized the critical nature of the angle of intercept between the two lobes which is essential in producing a high sheen hosiery yarn that does not have a garnishness related to excessive sparkle.

20 Additionally, when such multilobed forms are used in ladies' hosiery irrespective of the texturing method employed, three or more sizes of stretch hosiery are required to cover the range of consumer sizes. Indeed, to have truly satisfactory fits in stretch hosiery, five sizes 25 are judged by independent laboratories as being necessary to suit most consumer requirements for a comfortable and attractive fit.

20 There has been still another problem with prior art 30 yarns in that the stretch qualities on repeated stretching of hosiery results in continued loss of the original stress-strain properties and sagging or wrinkling of the hosiery may occur, particularly at the ankle section and knee section. With the foregoing discussion in mind, the provision for a homopolymer yarn which possesses the desired appearance factors as well as the desired stretch properties represents a substantial improvement in the art.

### SUMMARY OF THE INVENTION

40 The product of this invention involves a thermoplastic homopolymer fused into an oblong shape having two symmetrical lobes fused so that the concave sides intercept at an angle  $\theta$  ranging from 10 to 54°, and preferably at angle  $\theta$  42 to 52°, and 16 to 38°. The bifilament yarn has a broad concave area and a narrow edge (convex) area so that when said yarn is placed in a knit structure, the broad concave areas become aligned facing each other at stitch crossing points to present a convex or edge area to view and twist 90° or more to present the concave or broad areas to view in the loop sections. Light reflects from each concave area presented to view in the loop areas as a minute point flash and the alignment of these minute point flashes result in a sheen, opalescence, shimmer or scintillation point sometimes called "scintilla look" which is enhanced in bright yarns and reduced if a delusterant is present. Because of its geometrical configuration false-twist bifilament yarn has twice the number of point flashes; therefore, an enhanced luster or sheen is obtained in plain-knit hosiery.

45 Likewise, this twist trapped in each loop of the knitted structure gives greatly increased multidirectional elastic properties to the grid structure since each twist in each loop, coarse and wale becomes a multiple of the total number of loops of the grid structure thereby greatly enhancing its elasticity.

50 The preferred modification ratios are 1.65 to 3.0 and more preferably 1.75 to 2.8 and the most preferable 1.75 to 1.95 the tip radius is generally 0.9 or greater but less than 1.2. The bifilament yarns, textured and non-textured, semidull and bright, when converted to plain knit hosiery

as an undyed boardered structure have luster values as follows:

Bright non-textured: 9 to 40 ( $K/S \times 100$ ) units  
Bright false-twist: 12 to 45 ( $K/S \times 100$ ) units

These high luster values are due to alignment of minute point flashes resulting in a high glossy sheen termed the "glacé look" or "wet look" for bright yarns. This high sheen and uniform luster has not thus far been obtained in prior art knitted structures.

The preferred process for producing the yarn as above described involves employing a polyamide having a relative formic acid viscosity of between 25 and 90 which is extruded through a pair of spinnerette orifices having a distance between said orifices of 0.5 to 4.0 mils, preferably 1.0 to 3.5 mils. Nylon 6 is spun at a temperature of between 250 and 280°C., preferably 265 to 275°C., and nylon 6,6 is spun at approximately 10° higher temperature. The polyamide relative formic acid and the distance between the spinnerette orifices are the two major variables as indicated hereinafter in Table 1. With an increase in relative formic acid viscosity, the modification ratio increases and the angle of intercept decreases and the luster values increase. Thus, a sparkle look is produced and the desired high sheen "glacé look" is lost. It is noted, also, that the temperature of the polymer melt must be considered. As temperature increases, the modification ratio decreases. Additionally, at too high a temperature, drips, breaks and warps may appear, which are undesirable in the processing of such fibers.

Thermoplastics in general can be employed for producing bifilament yarns, but because of their excellent dyeing properties and good optical properties, polyamides usually are preferred for the production of bifilaments in accordance with this invention. Preferred polyamides are poly-*e*-caprolactam (nylon 6), polyhexamethylene adipamide (nylon 6,6), and the polyamides made by condensation of *p,p'*-bis(para-aminocyclohexyl)methane with dodecanedioic acid to produce the polyamide poly[bis(p-aminocyclohexyl)methane dodecamide].

The bifilament yarns disclosed as the invention herein also have utility in transport upholstery and apparel end uses because of the high elasticity of the knitted structure and the high glossy sheen or "glacé look" which characterizes knitted textile articles made from bright bifilaments.

#### BRIEF DESCRIPTION OF THE DRAWINGS

FIG. 1 is a cross section of the spinnerette orifices employed to extrude the bifilament yarns of the present invention.

FIG. 1A is a cross-sectional view representing the bifilament yarn of this invention illustrating how the angle of intercept  $\theta$  is measured.

FIG. 2 illustrates graphically the relationship between the optical properties of the filaments as a function of the angle of the bifilament intercept point versus the modification ratio.

FIG. 3 is a graph illustrating the lusture of bifilament yarns of this invention plotted against the modification ratio. These data illustrate the change in sheen between false-twist and normal yarn. The dotted lines show the range of modification ratio which produces the preferred high sheen yarn. The area to the right of the dotted lines shows the range of modification ratio which produces the "scintilla look."

FIG. 4 is a photograph illustrating, at 320 magnifications, representative cross sections of undrawn bifilament yarns of the instant invention which have a modification ratio of 1.7.

FIG. 5 is another photograph at 320 magnifications of other bifilament undrawn cross sections which have a high sheen "glacé look" when the yarn is placed in a sheer fabric. Generally, above this modification ratio of 2.0, a transition to the sparkle look occurs.

FIG. 6 is a photograph at 560 magnification of a typical cross section of drawn bifilament yarns having a modification ratio of 2.3 to 2.4, which illustrates the bifilaments of this invention.

FIG. 7 is a photograph at 900 magnifications of a drawn bifilament yarn having a modification ratio of 2.8 to 2.9, which produces the "scintilla look."

The yarns of FIGS. 6 and 7 are outside the critical range required to obtain a "glacé look."

FIG. 8 is a photograph illustrating the unique property obtained by combination of bifilament geometry with a false-twist operation. This illustrates the alignment of the concave surfaces at stitch cross-over points and the twist which in the loop part exposes the broad parts of the concave surfaces to view. This additionally illustrates the aligned rows of point light reflections from concave surfaces to give the unique sheen which can be observed. The magnification of FIGS. 8 through 13 is 36×.

FIG. 9 is a bifilament yarn in jersey knit hosiery which was not false-twisted. There is similar twist entrapment and alignment of the light reflective areas as in FIG. 8.

FIG. 10 is a photograph of a round cross-sectional yarn which is false-twisted and knit into hosiery. It can be observed that the light reflective areas are completely random, there is no twist between the stitches, and the yarn tends to curl back on itself rather than be twisted between the stitches.

FIG. 11 is a photograph of round monofilaments of plain knit hosiery. It also lacks the properties of twist entrapment and luster effects characteristic of bifilament yarns as illustrated in FIG. 9.

FIG. 12 is a photograph of stretch hosiery of round cross section, bicomponent filaments. Again, there is no alignment of the light areas in the yarn. Consequently, there is no luster or sheen, or enhancement of the elastically from twist trapped between stitches.

FIG. 13 is a photograph of mesh hosiery tuck stitch made from trilobal or triangular shaped yarns. As can be observed, the light reflection areas are random and significantly larger than those illustrated in FIGS. 8 and 9. Such yarns while suitable for many novelty end-uses have utility only as novelty yarns because of the garishness of the luster.

FIG. 14 is a graph illustrating the force required to elongate a bicomponent stretch yarn after one cycle of elongation, and, after six cycles of elongation. The stretch direction was lengthwise and the test sample was ladies' hosiery with plain knit construction.

FIGS. 15 and 16 represent the same test parameters as for FIG. 14 except that FIG. 15 represents false-twist bifilament yarns of this invention which have superior elastic properties over that for FIG. 14 and FIG. 16. FIG. 16 represents false-twist round cross section nylon 6 yarns.

FIGS. 17, 18 and 19 represent, respectively, leg sections of ladies' hosiery made from false-twist bifilament yarn, false-twist round filament yarns and round cross section bicomponent sheath and core yarn. The nature of the test data illustrated in these figures is similar to that described for FIGS. 14, 15 and 16, except the measurement is in the transverse direction.

#### DESCRIPTION OF THE PREFERRED EMBODIMENTS

The bifilament yarns of the present invention preferably are spun from a polyamide such as nylon 6 or nylon 6,6 directly from a continuous polymerization system wherein the polymers are melted prior to extrusion using an extruder or a melter. The molten polymer is then extruded through a pair of orifices in close proximity to each other as depicted in FIG. 1 by capillaries 1 and 3. These capillaries are separated by the portion 2 which is preferably an integral portion of the spinnerette plate 6. The molten polyamide polymer enters through an entry orifice denoted at 5 and is divided into separate streams

on contacting metallic portion 2. The distance between orifices 1 and 3 should be between 0.5 and 3.0 mils. The distance when less than 0.5 mil results in the separator portion or web 2, too weak to withstand the extrusion pressure. Should the distance between orifices 1 and 3 exceed 3.0 mils, one then enters the region of a sparkle effect and the preferred "glacé look" is not obtained. The length of spinnerette orifice 4 should generally be in the region of 0.8 to 4 times the diameter of the spinnerette orifices 1 to 3, preferably a length to diameter ratio of about 1.2 should be employed.

The yarn product of one part of the present invention has a "glacé look" which has been described as a "wet look" when fashioned into articles such as ladies' hosiery and other sheer garments. This appearance is achieved only when specific critical parameters are observed during the production of the bifilament yarns of this invention. It is essential that the yarns intercept at an angle of between 41 and 54° of the joined filaments. It is also preferred that the yarns have a modification ratio ranging from 1.65 to 2.05. At an intercept angle of greater than 54°, too low a luster is obtained and twist is not trapped between the filament loops to achieve the desirable elasticity properties in knit structures. At an angle of intercept below 41°, the yarn exhibits a sparkle effect and does not have the glacé look and desirable opalescent sheen of the product made in accordance with this invention.

The angle of intercept is determined by completing the two circles outlined by the filament lobes 12 and 14, then completing a line bisecting the center of the circles and the point where the circles intercept as shown in FIG. 1A. The angle of intercept is the angle  $\theta$  between the horizontal line passing through the center and the line drawn to the intercept point.

The modification ratio is determined by dividing the minimum width at the point of upper and lower intercept points of the two circles into the length or the distance to the outer perimeter of the two circles. The relationship between the angle and the modification ratio is given in FIG. 2 wherein it is illustrated that as the modification ratio decreases, the higher the angle of intercept.

As can be observed in FIG. 2, the glacé appearance coincides at an angle of intercept between approximately 38° and 56°, the area represented by ABCD. At a lower angle of intercept, the glacé look is lost and a sparkle effect occurs. At a broader angle of intercept than 54°, there is insufficient luster and the bifilaments lost most of their ability to align face to face at stitch cross-over points, the condition which imparts twist to said bifilaments in the loops between stitches. Therefore, they lose their luster, but most important, they lose their elasticity because of inability to trap twist between each stitch in the knitted structure. It is especially desirable that an angle of intercept be present on both sides of the bifilament yarns so that the twist is always trapped between stitches regardless of which side of the concave surfaces align at the stitch crossing points.

In FIG. 3 is shown a plot of the modification ratio versus luster. Luster is ascertained by measuring light reflectivity with a "Color Eye" manufactured by the Instrument Development Laboratories, Attleboro, Mass. The reflectivity is expressed by the Kubelka Munk equation where:

$$K/S = \frac{[1 - R]^2}{2R}$$

where R=reflectivity ascertained with the "Color Eye" at 557 millimicrons. The method for ascertaining the reflectance has been described in "Color and Business, Science and Industry" by D. B. Judd; John Wiley and Sons, New York, New York, 3rd printing, February 1967, pp. 434-438. As can be observed in FIG. 3, the luster values of significance are from 9 to 21 ( $K/S \times 100$ ) units, pref-

erably 10 to 18 ( $K/S \times 100$ ) units. For false-twist filament yarns, the luster values are quite significant higher than non-textured bifilament yarn made into hosiery. This is due to the presence of approximately twice as many concave reflection points in each stitch loop of textured over the non-textured bifilament yarn. Hosiery fashioned from the textured bifilament yarn have luster values of 14 to 21 ( $K/S \times 100$ ) units. The presence of this additional reflective surface or additional number of reflection points results in a considerable enhancement of the desirable "glacé look" over that obtained from the same hosiery made from non-textured bifilament yarns. This enhancement of the glacé look by a panel jury evaluation of skilled colourists amounts to 200 to 300 percent increase in the apparent sheen or luster values observed. Non-textured bifilament yarn has a luster value of 8 to 16 ( $K/S \times 100$ ) units. At lower values than the indicated range of bright luster, insufficient luster is present to produce a sheen effect at higher luster values, as, for example, greater than 16 for the non-textured and greater than 21 for the false-twist hosiery, there is excessive sparkle in the hosiery which tends to limit their utility to novelty end uses. Generally, within the scope of the luster values indicated, and as shown in FIG. 3, this hosiery is quite acceptable to be worn in everyday office use and still quite attractive and desirable for formal wear. The luster values for semidull yarns have the same modification ratio as bright yarns are quite different and only a low level of surface reflectivity is obtained. The major effect is a significant increase in cover due to the visual appearance of the broad concave surface in the loop section of the knitted structure. The increase in cover is 10-20 percent greater than round cross section yarn of the same denier.

A better appreciation for the critical influence that the angle of intercept and modification ratio of the yarn has upon appearance and the performance of the yarn of this product of this invention can be recognized from an investigation of FIG. 4 through FIG. 19. FIGS. 4 to 7 are photomicrographs of cross sections of bifilaments illustrating products of the invention compared with bifilament cross sections that are outside of the invention. The modification ratio of the cross sections shown in FIG. 4 is 1.7 and as can be observed there is only a slight distinct concave surface. Thus, the bifilaments having values below 1.5 and are not concave and generally have neither luster nor the elasticity desired. FIG. 5 is a cross section having a modification ratio of 2.0 which represents the upper limit beyond which excessive sparkle occurs. FIGS. 6 and 7 have modification ratios substantially greater than 2.0 and thereby representing yarns outside the scope of this invention.

FIGS. 4 and 5 illustrate the cross section of undrawn yarns and FIGS. 6 and 7 illustrate a cross section of drawn yarn. As can be observed, undrawn and drawn cross sections at equivalent magnification have identical geometric cross sections.

FIG. 6 is a photograph at 560 magnifications of a typical cross section of drawn bifilament yarn with a modification ratio of 2.3 to 2.4. Note that even though this is a view of random cross sections, there is a tendency for the bifilaments to align with the concave surfaces joining convex surfaces at maximum frictional contact.

FIG. 7 is a photograph at 900 magnifications of a drawn bifilament yarn having a modification ratio of 2.8 to 2.9. In the upper right hand corner can be observed alignment of the concave surface with the convex surface of essentially equal symmetry. This alignment provides for frictional resistance which entraps the twist in the loops and presents the narrow edge surface to view at stitch crossing points and thereby increase the sheerness of the hosiery or textile articles being employed. However, when the bifilament is in the loop section then the broad concave surface of the bifilament is in view and it is this broad surface that provides for additional cover in the delustered yarns.

Again, when referring to FIG. 1A and FIGS. 4 through 7, it can be noted that when the circle are completed, as indicated in FIG. 1A for circles 12 and 14, the total area of this circle is determined and their measured perimeter is divided into the perfect circle enclosing the measured area. From this arrangement their degree of circularity can be ascertained. Preferably the yarns of this invention have a degree of circularity of greater than 0.9. Bifilaments having a substantially larger deviation from circularity do not have the same sheen and knitting is difficult because of the tendency of such yarns to break out from back-up of twist at the needles.

The performance of hosiery fashioned from bifilament yarns made in accordance with this invention is compared with hosiery made from other yarns in FIGS. 8 through 19. These comparisons are made on the knitted structures since the unusual properties of light reflectivity and elasticity can be observed, and measured only after the yarn is placed in a fabric construction. It should be emphasized that hosiery is used as a common example; however, bifilament yarns react in a similar manner in other jersey knit structures, as well as, tricot knit structures, mesh or tuck stitch structures, and rib stitch structures.

FIG. 8 illustrates a section of hosiery fashioned from bifilament yarns having a modification ratio of 1.8. The yarn has 31 turns per inch of twist imparted thereto, utilizing a Leesona 553 Superloft machine. It is knitted into the hosiery using S and Z twist in alternate courses. It can be observed from FIG. 8, the light areas are short in length due to the twist of bifilament yarns between stitches; however, as can be noted, the light areas are all on an approximate similar plane. This results in a diaphanous, luminous sheen, which has been characterized as the "glacé look." As the modification ratio of bifilament yarns is increased, the length of the light flashes increases. As the intensity of the light at these points increases, each individual light-colored point results in a scintillation point, and the luminous sheen effect is replaced by a sparkle effect. Between each stitch it can be noted that the bifilament yarns twist 90 degrees first to present a flat plane to view and over the course of the twist, at least another 90 degrees for a total of at least 180 degrees to present two concave planes to view. It is this twist superimposed upon the false-twist stretch that lends sufficient elasticity to the hosiery so one size will span the range of sizes for most consumer end uses.

Additionally, as the stitches in FIG. 8 are stretched, the twist that is trapped between the stitches in the manner stated above gradually untwist and when tension is released, these twists rewind. After stretching, particularly in areas of hosiery where elongations ensue, that is, the areas which have greater propensity to sag or wrinkle, the twist which has been unwound as the individual stitches are stretched out, rewind into a normal configuration and provides additional force superimposed on that from the false-twist crimp. Thus, the combined forces, at low elongation, are adequate to hold the hosiery firm to the ankle or firm to the knee without any evidence of sagging or wrinkling. Moreover, such hosiery resists elongation on repetitive cycling.

In FIG. 9, a bifilament yarn the same as in FIG. 8, except without false-twist, illustrates that all light reflection areas are located at relatively precise points in the center of the plain-knit stitch and along the sides of the stitch. Thus, the bifils present the intercept point on a flat plane in the direction of the light and in the direction of the observer's view. In a comparison between the false-twisted and non-false-twisted yarns, it can be observed that the light areas and stitches are more uniform for the non-twisted yarn, and that the light areas are in a precisely aligned plane. It is this alignment of the reflection areas, which results in the smooth luminous sheen. This may be compared with round cross section yarn in FIG. 11 which exerts no twist entrapment and

5 has essentially no light reflective areas. Additionally, it may be compared with a trifilament yarn cross section in a mesh knit as illustrated in FIG. 13, where the point flashes extend over the long length of the tuck stitches and over broad areas of the standard jersey knit stitches. These broad areas of light reflection promote too much sparkle for most end uses, particularly for office wear and additionally as can be noted, there is less or no twist entrapment between stitches in FIG. 13.

10 FIG. 12 illustrates a time exposure for round cross section bicomponent elastic yarns. As can be observed, only small sparkle areas are obtained, and if it were not for the lengthy time of exposure, this sparkle could not be observed. Additionally, as can be observed, there is no twist entrapment between the stitches.

15 In FIG. 13 it can be observed that there is a bright sparkle in the center stitch. It is these large point sparkles that follow the entire length of the stitch which would seem to indicate there is relatively low level of change in planes of the reflecting surface. Therefore, no significant improvement in elastic properties or sheen could be expected from the yarn as illustrated in FIG. 13. Additionally, the sparkle is too bright except for formal occasions.

20 FIG. 14 illustrates the stress-strain characteristics of a plain knit hose manufactured from a commercial bi-component round fiber after one cycle and after six cycles. As can be observed, there is almost complete loss of a stretch power after six cycles, particularly at 3 percent elongation. Moreover, the values at 5 percent elongation are quite low. However, after these initial elongations there is a rapid increase in the gram loading for small increases in the elongation. It is this rapid increase which is undesirable because there is too much of a load for a given degree of stretch. This type of loading causes an uncomfortable effect on the part of the wearer as well as impart stresses to the individual filaments so that a sudden pick on impact will probably result in a run in the hosiery or garment.

25 FIG. 15 illustrates the lengthwise extension versus stress-strain load for a hose constructed the same as in FIG. 14 except the bifilament yarn of this invention which has been false-twisted was employed. As can be noted, the hose has a definite initial loading that is still high after six cycles of extension which slopes upward at a substantially lower rate than that described in FIG. 14. Thus, it has a relatively uniform stretch characteristic maintaining a definite power after repetitive stretching sufficient to avoid wrinkling or sagging of the hosiery.

30 FIG. 16 represents hosiery processes in identical manner to that illustrated in FIG. 15 with the only difference being round cross section versus bifilament yarns. Again at 3 percent elongation, after six cycles, there is no power left in the yarn and sagging or wrinkling can occur. Additionally, there is considerable greater drop in the load at 5 percent elongation from the first to the sixth cycle. Generally there is a slower increase in loading with a substantial increase in elongation for the round false-twist yarn than that for the bifilament yarn, as illustrated in FIG. 15, when tested in a lengthwise direction.

35 False-twist triangular or trilobal cross section yarn is converted into hosiery and processed in identical manner to that as illustrated in FIG. 15 with the only difference being round cross section bifilament yarn versus the round cross section of FIG. 16. Again this cross section exhibits very low load capacities after six cycles which is similar to that for round cross section false-twist yarn, except that at 10 percent elongation and above, loading is very rapid, even more rapid than that illustrated in FIG. 15. This would cause an uncomfortable effect on the part of the wearer as well as stress individual filaments to increase the potential of runs or breakage of the filament from sudden picks or impact.

FIG. 17 illustrates a bifilament yarn in the transverse direction. Comparing FIG. 17 with FIG. 15, it can be observed generally there is a far lower increase in loading in the transverse direction for a given degree of elongation than there is in the lengthwise direction. It is, however, an unexpected advantage of the bifilament yarn, that it has a definite and significant loading capacity even at elongations as low as 3 percent which still remain adequate after six cycles of extension.

FIG. 18 shows exactly the same transverse stress-strain curve for a false-twisted round cross section yarn. As can be noted at low elongation, 3 to 5 percent after six cycles, the false-twist yarn has essentially no load-bearing capacity. Therefore, it would tend to wrinkle. In a similar manner, a triangular cross section false-twisted yarn shows essentially the same initial transverse stress-strain curve as that for round cross section, and then very rapidly loads which is an indication of limited and narrow elastic characteristics.

FIG. 19 illustrates a bicomponent yarn in a transverse extension. This yarn also has very low load-bearing capacities throughout the range tested up to 25 percent elongation. Again, if wrinkling should occur, it more probably would occur with the bicomponent yarn of FIG. 19 than with yarn of FIG. 18, and especially with yarn of this invention illustrated in FIG. 17.

From the foregoing illustrations and comparisons made in connection with the drawings, it can be seen that, in general, the luster of bifilament yarns is a function of the modification ratio whether a "glacé look" or a sparkle effect is obtained. Other configurations show quite different luster effects and do not normally demonstrate the silky high sheen characteristic of the modification ratios of between 1.65 and 2.0, and 2.05 to 3.0 which are illustrated in FIGS. 2 and 3. Many end-uses of knit apparel structures require a low degree of transparency. To achieve this effect, anatase titanium dioxide is dispersed in the monomer or at some point prior to completion of the polymerization cycle in the amount of 0.3 percent of  $TiO_2$  by weight of polymer for semidull articles and 2.0 percent by weight of  $TiO_2$  by weight of polymer for full-dull articles. This delustering quality is desirable for its hiding power, but frequently it has undesirable chalkiness or grayishness which decreases the aesthetic properties of the textile article containing said delustrant. Thus, when the bifilament yarn of this invention is made into knit textile articles, an enhanced warmth of appearance and aesthetic properties is obtained. The delustered yarn has 10-20 percent greater cover on a standard hosiery form as compared with round cross sections of equivalent denier. The high luster obtained for bright yarn has the further advantage in that the high degree of reflectivity which is obtained significantly reduces the apparent soiling as compared with round cross sections and triangular cross sections.

The following examples further illustrate the invention.

#### EXAMPLES 1-14

The bifilamentary yarns of the present invention were prepared from polycaproamide pellets of 50 to 65 relative formic acid viscosity which were spun at a temperature of 255 to 270° C. from a melter through twin spinnerette orifices, 10 mils in diameter by 10 mils in length and separated from each other at a minimum distance of 2 mils. The metal web separating the two spinnerette orifices was counterdrilled from the spinnerette face for a distance of 3 mils. The spinnerette employed had a counterbore angle of 60° as indicated by reference numeral 5 in FIG. 1. The molten polymer entered the spinnerette counterbore at the rate of 4.78 grams/minute/bifil filament. There were four spinnerettes per stack, each spinnerette producing two strands of bifilament yarn and each spinnerette was separately metered. Thus, eight strands of bifilament yarn were produced per quench stack. The yarn

was quenched 3 inches below the spinnerette face with quench air entering at the temperature of from 20° C. to 41° C. and traveled uniformly transverse to the filaments, at the rate of 10 lineal feet/min. for a distance of 95 inches from the point of initial gas contact with the filaments. The yarn then entered a round quench stack of about 7 inches in diameter, thence over a lubrication roll where finish was applied at about 8 to 10 percent by weight of yarn. The yarn was then taken up on a winder having two cops per sleeve and using four sleeves per winder making a total number of eight ends per winder having 4.7 pounds/cop or 9.4 pounds/sleeve. The speed of take-up was 1,950 feet/min. for the undrawn yarn. The bifilament yarn was then placed on drawtwisters 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 101

The true visual rating for the increase in sheen for the false-twist bifilament yarns as compared with the non-textured bifilament yarns was 200 to 300 percent greater at equal extension of a standard hosiery leg form. The panel jury of experienced colourists rated the bifilament yarns of this invention as having a sheer appearance value equal to between 10 to 12 denier for the 20 filament bi-

The Instron was equipped with G61-3C air-operated clamps gripping for a distance of 2 inches and the two jaws were separated from each other by a distance of 2 inches in lengthwise tests and 1 inch in the transverse tests. The rate of elongation was at 10 inches per minute on the loading part of the cycle and at the same rate on the unloading part of the cycle.

TABLE 1.—OPTICAL OR LUSTER PROPERTIES AS MEASURED ON THE BOARDED HOSIERY

| Example No. | ( <sup>1</sup> 2) | Type cross section | Modification ratio | Angle of bifilament intercept degrees | Percent <sup>3</sup> luster K/S by "color eye"          | Panel jury <sup>4</sup> Rating of the degree of silky sheen "glacé look" |
|-------------|-------------------|--------------------|--------------------|---------------------------------------|---------------------------------------------------------|--------------------------------------------------------------------------|
| 1           | Br                | Bifilament         | 1.4                | 62                                    | 6.0                                                     | No sheen, similar to round.                                              |
| 2           | Br                | do                 | 1.65               | 55                                    | 10.0                                                    | Good (A) subdues sheen.                                                  |
| 2A          | SD                | do                 | 1.70               | 52.5                                  | 10-20% greater cover over Example 6A.                   |                                                                          |
| 3           | Br                | do                 | 1.8                | 49.2                                  | 12.0                                                    | Excellent strong "glacé look" high sheen.                                |
| 3A          | SD                | do                 | 1.95               | 44                                    | 10-20% greater cover compared with Example 6A.          |                                                                          |
| 4           | Br                | do                 | 2.0                | 42.5                                  | 14.0                                                    | Good (B) "glacé look" with slight sparkle.                               |
| 4A          | Br                | do                 | 2.8                | 17                                    | 33.3                                                    | Good (B) heavy point sparkle.                                            |
| 5           | Br                | do                 | 2.5                | 27                                    | 24.0                                                    | No "glacé look", definite sparkle.                                       |
| 5A          | Br                | do                 | 3.1                | 9                                     | (6)                                                     | Splits and excessive sparkle higher.                                     |
| 6           | Br                | Round              | 1.0                | 4.5                                   | No "glacé look".                                        |                                                                          |
| 6A          | SD                | do                 | 1.0                | 45.0                                  | Dull without warmth.                                    |                                                                          |
| 7           | Br                | Triangular         |                    |                                       | Heavy sparkle, too garish for most end-uses in hosiery. |                                                                          |
| 7A          | Br                | F-T triangular     |                    |                                       | Heavy "sparkle".                                        |                                                                          |
| 8           | Br                | F-T bifilament     | 1.7                | 52.5                                  | 15.5                                                    | Good (A) subdued "glacé look".                                           |
| 8A          | SD                | do                 | 1.8                | 49.2                                  | Subdued sheen.                                          |                                                                          |
| 9           | Br                | do                 | 1.9                | 46                                    | 18.0                                                    | Excellent strong "glacé look".                                           |
| 9A          | Br                | do                 | 2.8                | 17                                    | 40.0                                                    | Excellent strong iridescent point sparkle "scintilla look".              |
| 10          | Br                | do                 | 2.05               | 41                                    | 12.0                                                    | Subdued warm sheen.                                                      |
| 10A         | Br                | do                 | 3.0                | 10                                    | 44.0                                                    | Good (B) heavy point sparkle.                                            |
| 11          | Br                | F-T Round          | 1.0                | 3.5                                   | No "glacé look".                                        |                                                                          |
| 12          | Br                | F-T bifilament     | 2.5                | 42                                    | 23.0                                                    | No "glacé look", definite sparkle.                                       |
| 12A         | Br                | do                 | 1.9                | 46                                    | 16.5                                                    | "Glacé look", too low a sparkle for scintilla look.                      |

<sup>1</sup> Br=Bright hosiery. <sup>2</sup> (Delustrant) SD=Semi dull=0.3% by weight anatase TiO<sub>2</sub>.

<sup>3</sup> Luster is measured on the white boarded hosiery before dyeing.

<sup>4</sup> The panel jury of 5 experienced colourists' rating is based on observation of the dyed hosiery, and is as follows: Excellent=Opalescent smooth silky high sheen, the preferred "glacé look"; Good (A)=Opalescent silky sheen "glacé look" present but slightly subdued; Good (B)=An opalescent high sheen with the preferred "glacé look" but some sparkle present.

<sup>5</sup> Too non-uniform to read.

NOTE. E-T=False twist.

TABLE 2.—FORCE IN GRAMS FOR HOISERY EXTENDED LENGTHWISE AT THE INDICATED ELONGATIONS<sup>1</sup>

| Example No.                                                               | Number of cycles | Percent work of recovery | Ankle elongation, percent |       |       |       |       | Knee elongation, percent |      |       |     |     |       |
|---------------------------------------------------------------------------|------------------|--------------------------|---------------------------|-------|-------|-------|-------|--------------------------|------|-------|-----|-----|-------|
|                                                                           |                  |                          | 3                         | 5     | 10    | 15    | 20    | 25                       | 3    | 5     | 10  | 15  |       |
| 9. Bifil false-twist standard knit stretch hosiery <sup>2</sup>           | 1                | 59.3                     | 18                        | 27    | 48    | 78    | 113   | 145                      | 58.3 | 18    | 22  | 32  | 45    |
|                                                                           | 6                | 64.2                     | 10                        | 16    | 34    | 63    | 100   | 136                      | 63.2 | 8     | 12  | 23  | 36    |
| 11. Round filament false-twist standard knit stretch hosiery <sup>2</sup> | 1                | 43.7                     | 14                        | 20    | 40    | 63    | 87    | 113                      | 54.0 | 12    | 17  | 30  | 47    |
|                                                                           | 6                | 50.5                     | 2                         | 5     | 22    | 43    | 72    | 103                      | 56.4 | 3     | 7   | 19  | 36    |
| 13. Bicomponent standard knit stretch hosiery <sup>2</sup>                | 1                | 44.6                     | 18                        | 25    | 50    | 6     | 137   | 200                      | 53.2 | 18    | 25  | 45  | 72    |
|                                                                           | 6                | 48.2                     | 4                         | 12    | 32    | 67    | 121   | 195                      | 58.1 | 7     | 12  | 30  | 66    |
| 7A. Triangular cross section false-twist <sup>2</sup>                     | 6                | 52.0                     | 1                         | 5     | 25    | 50    | 80    | 105                      | 47.1 | 1     | 3   | 12  | 22    |
| 3. Bifilament cross section standard knit hosiery, Nylon 6 <sup>2</sup>   | 1                | 4.4                      | 300                       | 400   | 800   | 1,200 | 1,700 | 2,300                    | 45.0 | 300   | 500 | 850 | 1,320 |
|                                                                           | 6                | 59.0                     | 50                        | 60    | 300   | 700   | 1,300 | 2,100                    | 60.4 | ----- | 50  | 350 | 800   |
| 6. Round cross section standard knit hosiery, Nylon 6 <sup>2</sup>        | 1                | 39.0                     | 400                       | 650   | 1,300 | 2,000 | 2,800 | 3,600                    | 41.0 | 300   | 500 | 950 | 1,350 |
|                                                                           | 6                | 56.0                     | (3)                       | 50    | 400   | 1,100 | 2,100 | 3,300                    | 52.2 | ----- | 50  | 450 | 880   |
| 14. Bifilament cross section mesh-knit, Nylon 6 <sup>4</sup>              | 1                | 40.6                     | 450                       | 800   | 2,000 | 3,400 | 5,000 | 6,500                    | 45.7 | 200   | 350 | 650 | 1,100 |
|                                                                           | 6                | 57.5                     | (3)                       | (3)   | 500   | 1,800 | 3,700 | 6,200                    | 61.2 | ----- | 300 | 600 | 1,300 |
| 7. Triangular cross section mesh-knit, Nylon 6,6 <sup>4</sup>             | 1                | 38.7                     | 500                       | 1,000 | 2,200 | 3,520 | 4,900 | 6,250                    | 41.1 | 200   | 320 | 700 | 1,200 |
|                                                                           | 6                | 58.5                     | (3)                       | (3)   | 400   | 1,700 | 3,600 | 5,800                    | 58.8 | ----- | 200 | 600 | 1,350 |

<sup>1</sup> The values in the table are all expressed in grams with the exception of work of recovery.

<sup>2</sup> Standard knit, plain or jersey stitch.

<sup>3</sup> Load too small to show on chart.

<sup>4</sup> Mesh knit=tuck stitch.

<sup>5</sup> Too small to read on Instron on 10,000 gram load scale.

filament. This property is of significant value since it means that the bifilament yarns have an improvement in sheeress values of 165 percent without a loss in wearing properties as would normally be expected with a corresponding reduction in the denier typically required in round cross section hosiery to achieve the present sheeress values.

The improvement in sheeress is due to alignment of the concave surfaces facing each other at stitch crossing points so as to present the narrow edge to view.

All luster values listed in Table 1 were ascertained using a color eye fabric sample holder with a black background and employing a Model D-1 "Color-Eye."

The boarded stockings were dyed in a conventional manner, dried by the tray method and placed in an Instron tester to evaluate the stretch properties of the hosiery. The hosiery were pretensioned at 1 percent of the total Instron loading which was 100 to 500 grams minimum and 2,000 grams maximum. Thus, the pretensioning was between 1 to 5 and 20 grams, depending upon the degree of stretch in the hosiery being tested and the loads required to elongate the hosiery to 25 percent.

Work of recovery is the ratio of recoverable work to the total work required to strain a fiber or fabric a specified amount under a given program of strain rate. In this case, it was determined at 25 percent elongation 15 seconds forward cycle, 15 seconds return and was calculated according to ASTM D-1774-64, ASTM Standards (1964) part 25, pp. 428-432.

All values for Tables 2, 3, 4 and 5 were measured using Instron G61-3C 2-inch rubber faced air operated jaws clamped with 60 pound pressure. The cross head and gage length were the same and a 25 percent elongation was achieved in 15 seconds. There were 2 inches of hosiery between the clamped jaws and lengthwise tests and 1 inch of hosiery between clamped jaws in the transverse or width tests.

The bicomponent and triangular yarns evaluated herein are sold commercially.

The elastic properties of the hosiery on lengthwise extension are given in Table 2. As can be seen the ankle and the knee areas were selected since these are the areas of greatest wrinkle problems in ladies' hosiery.

Referring to the results shown in Table 2, it can be

noted that the bifilament false-twist yarns have the highest work of recovery of all yarns tested and the improvement in terms of work of recovery is the greatest after 6 cycles when compared to other types of yarns tested as indicated by Example 9. Most significant in the stress-strain curve was the stress force at an elongation of 3 percent. It can be noted that the hosiery of Example 9 had a stress force of 16 grams which was 250 to 500 percent higher loading in the ankle area at 3 percent elongation than the round cross-section false-twisted yarn (Example 11) or bicomponent stretch hosiery (Example 13). Without false twist, the bifilament cross section, plain knit or jersey knit hosiery (Example 3) may be compared with the round cross section yarn (Example 6). The work of recovery on the first cycle is 44.4 percent or 10 percent higher for the bifilament cross section than the round which would indicate definitely improved wrinkle resistance. In Table 2, it can be observed further that the bifilament cross section yarn (Example 3) has a greater elasticity after 6 cycles of extension than the round cross section of plain knit and less force is required to extend it to 25 percent. Indeed, the stress forces are about  $\frac{1}{2}$  that required to extend round cross section yarn of an equal denier. After six cycles of extension the bifilament cross section plain knit hosiery has a stress force of 50 grams which indicates excellent capacity to retain its shape, whereas the round cross section has an immeasurably small value.

Bifilament yarns containing 0.3 percent  $TiO_2$  and 2 percent  $TiO_2$  were converted to false-twist yarns similar to that described for Example 9 and exhibited similar elastic properties in test hosiery as that illustrated in Table 2 for Example 9. Likewise, bifilament cross section yarns containing 0.3 and 2.0 percent of  $TiO_2$  were converted to standard jersey knit hosiery. The bifilament yarns containing  $TiO_2$  exhibited similar elastic properties as that of Example 3. The bifilament false-twist yarn of Example 9 might be additionally compared with the triangular cross section false-twist yarn of Example 7A in the form of similar hosiery. As can be observed, the work of recovery for the triangular cross section false-twist yarn is significantly less than bifil false-twist yarns and the elongation after six cycles at 3 percent elongation was 1 gram compared with 10 grams, or about 10 percent of that obtained for the bifilament yarns at the ankle section of the hosiery.

Likewise, the triangular cross section yarn hosiery in the knee section had significantly less work of recovery and very low load to 0 loads at 3 percent elongation than did the bifilament cross section of Example 9 which had a stress force of 9 grams when tested in the knee section. Thus, it should be expected that the triangular cross section yarns generally would have greater problems with sagging and wrinkling than would the bifilament yarns of this invention.

Examples 14 and 7, respectively, show a comparison of bifilament cross section with triangular cross section in a mesh knit stocking. Generally, the elastic properties are approximately equivalent to the triangular cross section in the mesh knit hosiery. It is believed that failure to show equivalent advantages here may be due to tuck knit stitch on long courses having reduced twist and,

consequently, this type stitch interferes with the ability of this yarn to twist at stitch doubling areas.

The data for Examples 9, 11 and 13 are shown graphically in FIGS. 15, 16 and 14, respectively, and the picture of the knit hose of Example 9 is shown in FIG. 8, Example 11 in FIG. 10, and Example 13 in FIG. 12.

The bifil cross section mesh knit hosiery has 5 to 10 percent greater work of recovery in the knee section than does triangular cross section mesh knit yarn, both being made employing a tuck knit stitch. After six cycles, the bifil cross section appears to retain 50 percent more force in the knee section at 10 percent elongations. However, in Table 3, it can be observed that in the transverse direction, the bifilament mesh knit hosiery after six cycles, has a stress force of 10 grams at 3 percent elongation and at the knee section and at the welt section. Additionally, after 6 cycles, the power of recovery (see Table 4) of the bifil mesh knit in the lengthwise knee area was 150 grams or 150 percent greater than that for the triangular cross section.

In Table 3, bifilament false-twist yarns (Example 9) are superior to round false-twist yarns (Example 11) and bicomponent round cross section (Example 13) in plain knit in a transverse direction over the entire range of elongation and at 25 percent elongation, especially after 6 cycles of extension. The values vary between 200 percent and 100 percent higher for Example 9 than for Examples 11 and 13 in the transverse direction. For bifilament plain knit hosiery (Example 3) as compared with round plain knit standard hosiery (Example 6) it can be observed that the transverse force elongation values are much higher and would represent a more comfortable extension force than that obtained for round cross section. After 6 cycles, the values for the bifilament were adequate to avoid wrinkling and obtained a smooth fit in the ankle region and in the knee region.

Example 7A, triangular cross section false-twist yarns had similar properties in transverse direction to that of the bicomponent yarns up to a 10 percent elongation; however, at 10 percent elongation and above, very rapid loading ensued which indicated a lower degree of elasticity for the triangular cross sections of this yarn.

Table 4 illustrates a more significant part of the elastic properties. In this case the yarn was extended to 25 percent elongation and allowed to return to  $12\frac{1}{2}$  percent elongation and the force in grams ascertained at this point by reading from the chart. This value is designated as the "power of recovery," and is frequently referred to as the muscle power of the fabric and is probably a more significant value than is the forward extension part of the cycle. As can be observed in Table 4, bifilament false-twist stretch hosiery (Example 9) after six cycles of lengthwise strength has a power of recovery of 25 grams or 300 percent greater force at the ankle as compared with the bicomponent round cross section false-twist stretch yarn. Additionally, the bifilament yarn has significantly higher values in the knee section.

In Example 9, bifilament false-twist stretch hosiery after six cycles of lengthwise stretch has at least 200 percent greater force at the ankle as compared with a triangular cross section (Example 7A) false-twist stretch hosiery of identical construction.

TABLE 3.—HOSEY PHYSICAL PROPERTIES—TRANSVERSE

| Example No.                                    | Number of cycles | Ankle elongation, percent |    |     |     | Below-welt-thigh area elongation, percent |    |     |     |
|------------------------------------------------|------------------|---------------------------|----|-----|-----|-------------------------------------------|----|-----|-----|
|                                                |                  | 3                         | 5  | 10  | 25  | 3                                         | 5  | 10  | 25  |
| 9. Bifil F.T. <sup>1</sup>                     | 6                | 5                         | 7  | 12  | 50  | 5                                         | 7  | 15  | 60  |
| 11. Round F.T. <sup>1</sup>                    | 6                | 1                         | 3  | 5   | 26  | 2                                         | 7  | 7   | 50  |
| 13. Bicomponent <sup>1</sup>                   | 6                | —                         | 3  | 6   | 15  | 3                                         | 5  | 10  | 25  |
| 7A. Triangular cross section F.T. <sup>1</sup> | 6                | 2                         | 5  | 125 | 3   | —                                         | —  | —   | —   |
| 3. Bifil plain <sup>1</sup>                    | 6                | 5                         | 10 | 50  | 190 | 5                                         | 70 | 550 | —   |
| 6. Round cross section <sup>1</sup>            | 6                | 4                         | 10 | 100 | 470 | 5                                         | 80 | 460 | —   |
| 14. Bifil mesh knit <sup>2</sup>               | 6                | 5                         | 10 | 40  | 380 | 10                                        | 10 | 30  | 570 |
| 7. Triangular mesh knit                        | 6                | 5                         | 10 | 35  | 185 | 5                                         | 8  | 25  | 270 |

<sup>1</sup> Plain or jersey knit.<sup>2</sup> Mesh knit or tuck stitch hosiery.

NOTE.—F.T.=False twist.

A similar improvement for Example 9 over Example 11 and Example 13 can be observed for the "power of recovery" in the transverse direction. The power of recovery for bifilament yarn (Example 3) in the knee section is 125 grams or approximately twice that of the round cross section (Example 6) in the lengthwise direction. The power of the recovery of 175 grams for bifilament cross section mesh knit yarn (Example 14) is approximately twice that for the triangular cross section mesh knit hosiery (Example 7) after 6 cycles of extension.

It is observed that the bifilament yarns (Examples 2, 3, 8, 9 and 10) in a 20-denier exhibited approximately the same sheerness of that observed for a 10-denier monofilament. This is because bifilament yarns where they cross at the stitch point present the narrow edge of the filament to view. Thus, at the point of maximum abrasion or compression one presents the best geometric area for breaking resistance while the minimum geometric area is presented to the eye, thereby achieving sheerness and simultaneously good wearing qualities of the hosiery.

Panel jury tests of 20 women in wear tests of a single

TABLE 4.—"POWER OF RECOVERY"—EXTENSION TO 25% ELONGATION WITH MEASUREMENT OF LOAD ON RETURN TO 12½% ELONGATION

| Example No.                                           | Number of cycles | Lengthwise of hosiery <sup>1</sup> |      |       | Transverse or width direction of hosiery <sup>1</sup> |      |       |
|-------------------------------------------------------|------------------|------------------------------------|------|-------|-------------------------------------------------------|------|-------|
|                                                       |                  | Ankle                              | Knee | Thigh | Ankle                                                 | Knee | Thigh |
| 9. Bifil false-twist <sup>2</sup>                     | 1                | 27                                 | 20   | 10    | —                                                     | —    | —     |
|                                                       | 6                | 25                                 | 15   | 7     | 10                                                    | 8    | 7     |
| 11. Round cross section false-twist <sup>2</sup>      | 1                | 14                                 | 12   | 7     | —                                                     | —    | —     |
|                                                       | 6                | 8                                  | 8    | 5     | 3.5                                                   | 3    | 3     |
| 13. Bicomponent round cross section <sup>2</sup>      | 1                | 12                                 | 18   | (3)   | —                                                     | —    | —     |
|                                                       | 6                | 7                                  | 12   | (3)   | 3.5                                                   | 5    | 5     |
| 7A. Triangular cross section false-twist <sup>2</sup> | 6                | 12                                 | 7    | —     | —                                                     | —    | —     |
| 3. Bifil hosiery <sup>2</sup>                         | 1                | 250                                | 150  | 130   | —                                                     | —    | —     |
|                                                       | 6                | 150                                | 125  | 100   | 20                                                    | 40   | 50    |
| 6. Round hosiery <sup>2</sup>                         | 1                | 225                                | 100  | 60    | —                                                     | —    | —     |
|                                                       | 6                | 150                                | 60   | 50    | 30                                                    | 20   | 10    |
| 14. Bifil mesh knit                                   | 1                | 350                                | 200  | 350   | —                                                     | —    | —     |
|                                                       | 6                | 250                                | 175  | 250   | 35                                                    | 26   | 26    |
| 7. Triangular mesh knit sparkle yarn                  | 1                | 300                                | 150  | 150   | —                                                     | —    | —     |
|                                                       | 6                | 200                                | 100  | 125   | 25                                                    | 20   | 12    |

<sup>1</sup> Force in grams after extension to 25% elongation and return to 12½% elongation is designated the "power of recovery".

<sup>2</sup> Plain or jersey knit.

<sup>3</sup> No data.

Table 5 illustrates the maximum elongation of stretch hosiery at fixed stress loads. As can be observed in Table 5, Example 9 bifilament false-twist stretch hosiery were superior to round cross section false-twist stretch hosiery (Example 11) and Example 13 bicomponent round cross section stretch hosiery. It can be noted on a single cycle that both false-twist yarns were substantially superior to bicomponent round stretch hosiery in their total elongation. Thus, it can be concluded that the major differences between the two cross sections are best illustrated after repetitive cycling.

TABLE 5.—MAXIMUM ELONGATION OF HOSIERY, STRETCH AT ANKLE

| Example No.                           |   | Percent elongation, after one cycle |           |                                        |           |
|---------------------------------------|---|-------------------------------------|-----------|----------------------------------------|-----------|
|                                       |   | 500                                 | 1,000     | Where yield point occurs <sup>51</sup> | 2,000     |
|                                       |   | gram load                           | gram load | gram load                              | gram load |
| 9. Bifil false-twist stretch hosiery  | — | 85                                  | 101       | 84                                     | 120       |
| 11. Round false-twist stretch hosiery | — | 84                                  | 98        | 80                                     | 118       |
| 13. Bicomponent round stretch hosiery | — | 36                                  | 56        | 36                                     | 80        |

<sup>1</sup> This value was obtained in the test procedure similar to that for the yield point in yarns where a straight line is taken along initial load line, then a similar straight line is drawn at maximum loading or stress to bisect the first line drawn and then a straight line from this intercept with the stress-strain line drawn by the Instron. This intercept point is called the "Yield Point."

From Tables 2 through 5 the following general conclusions may be drawn:

(1) Bifilament false-twist yarns (Example 9) on repetitive cycling have substantially improved elastic properties as compared with Examples 11, 7A and 13 over the entire range of tests evaluated.

(2) Bifilament cross section yarn in standard knit hosiery (Example 3), as compared with round cross section in standard knit hosiery, has some slightly improved properties after 1 cycle and significantly improved properties after 6 cycles over the entire range evaluated.

(3) Bifilament cross section mesh knit hosiery (Example 14) has equal properties over most tests employed and slightly to significantly improved properties after 6 cycles of testing as compared with a triangular cross section mesh knit hosiery.

size hosiery made of false-twist bifilament yarns (Example 9) rated them as sag-free having excellent wearing qualities and having exceptional aesthetic qualities in appearance. They rated the comfort fit over an entire range of leg sizes of 8½ to 10½ as excellent. The wearing qualities were quite superior to other hosiery such as Example 11, false-twist round cross section hosiery, Example 7A triangular cross section false-twist hosiery, and Example 13 bicomponent standard knit stretch hosiery. The bicomponent hosiery in all examples were composed of nylon 6,6 as the sheath portion which is about 35 percent by weight and nylon 6,10-6,6 copolymer in the core portion generally in the kidney shape as 65 percent of the total.

The above hosiery fashioned from bicomponent and triangular cross-section yarns were purchased for comparative evaluations.

#### EXAMPLE 15

Bicomponent yarn was prepared by the procedures described in Examples 1-14 except nylon 6,6 was employed. The bifilament yarn was false-twisted and compared with similar hosiery made from false-twist round cross section yarn. These were tested for work of recovery, and stress-strain curves similar to those indicated in Tables 2, 3, 4 and 5. The bifilament hosiery made from polyhexamethylene adipamide showed approximately equivalent improvement in all physical properties and in luster effects as that already described for polycaprolactam when compared with the round cross section made under identical conditions except with respect to the spinnerettes employed. The spinning temperature was maintained at about 280° C. to produce a galcé look from the polyhexamethylene adipamide (nylon 6,6).

#### EXAMPLE 16

Poly[bis(para-aminocyclohexyl)methane dodecamides] was spun at a temperature of 290° C. through bifilament spinnerettes of the type illustrated in FIG. 1 and was drawn at a draw ratio of 3. The drawn yarn had a density of 1.001; a moisture absorption of 3 percent at 65 percent relative humidity and a glass transition temperature of greater than 100° C. This yarn was also prepared

in round cross section. The same improvement in elastic properties for bifilament cross section in hosiery after twisting over the control in round cross section was noted; however, the elastic properties as compared with polycaproamide and polyhexamethylene adipamide was approximately twice as great in the force in grams at low elongations of 3 and 5 percent. The work of recovery was between 10 and 15 percent higher than that indicated for polycaproamide. The muscle value or power of recovery was approximately 100 percent greater than the polycaproamide listed as Example 9, Table 4, for the ankle, knee and thigh dimensions.

These values are desirable for support hosiery but too high for conventional stretch hosiery, for a comfortable fit.

#### EXAMPLE 17

A series of runs was made employing polyamides of relative formic acid viscosity of 25 to 90 using a spinnerette of the type illustrated in FIG. 1. A range of temperatures from 250 to 290° C. were evaluated. The distance between the spinnerette orifices tested was from 0.9 to 4.0 mils. Heated quench air immediately below the spinnerette was evaluated in the range of 260 to 350° C. and the velocity of the quench air in the vicinity of  $\frac{1}{4}$  to  $\frac{1}{2}$  inch from the spinnerette face was evaluated in the range of 0 to 8 standard cubic feet/minute/25 pounds per hour throughput. Polymer throughput was evaluated at a high rate, 8 grams/minute/bifilament and at a low rate of 2 grams/minute/bifilament. The spinnerette orifice length of 20 to 150 mils was evaluated.

In Table 6 are the results of these evaluations in order to optimize the "glacé look."

The web separating the twin capillaries was counterbored from the spinnerette face for a distance of 5 mils to provide initial molten stream contact and avoid bifilament splits at high modification ratios. The spinnerettes employed have straight-sided counterbore. Normally, no heat is required in the vicinity of spinnerettes, but in this case, it is desirable to have a high melt viscosity polymer and small spinnerette orifices. Thus, the role of the heated ring is for good spinnability and to avoid splits due to irregular movement of the yarn at the capillary exit.

The yarn was contacted approximately 9 inches below the spinnerette by 200 cubic feet/min. of gas which was diffused into the quench stack for a distance of 2 feet along the outer peripheral of the 48 inch quench stack so that the maximum lineal velocity of the quench gas is 8 feet/min. Thirty cubic feet/min. of gas is exhausted upwards countercurrent to the flow of the filaments and out through monomer exhaust ports, located approximately even with the spinnerette. A distance of  $\frac{1}{4}$  to  $\frac{1}{2}$  inch separated the spinnerette face from the resistance heating ring. The velocity of the exhaust gas was less than 2 lineal feet/min. The quench gas then travels cocurrent with the filament and was exhausted at a point approximately 17 feet below the spinnerette face. The 168 ends of yarn were passed over a single finish roll grooved to act as a guide for the 168 ends. To each filament was applied 8 to 10 percent by weight of finish emulsion equal to about 1 percent of finish oils. The yarn then contacted a take-up roll having a peripheral speed equal to 1000 ft./min. and thence passed over draw rolls traveling at a lineal speed of 4,000 feet/min. Three wraps were taken on the draw roll and three wraps were taken on the take-

TABLE 6.—PROCESS FOR CONTROL OF MODIFICATION RATIO

|                                                             | Significance level | Approximate relative effect <sup>1</sup> | Assuming value <sup>2</sup>        | "Glacé look" | "Scintilla look" |                        |           |
|-------------------------------------------------------------|--------------------|------------------------------------------|------------------------------------|--------------|------------------|------------------------|-----------|
|                                                             |                    |                                          |                                    | Range        | Preferred        | Range                  | Preferred |
| Polyamide relative formic acid viscosity.....               | 1                  | 100                                      | Increases.....                     | 25-65.....   | 40-60.....       | 40-90.....             | 58-75     |
| Mils between spinnerette orifices.....                      | 2                  | 90                                       | do.....                            | 0.9-3.0..... | 1.5-2.5.....     | 2.5-4.0.....           | 2.5-3.5   |
| Temperature, °C.....                                        | 3                  | 60                                       | Decreases.....                     | 270-280..... | 265-275.....     | 255-290.....           | 260-280   |
| Heated quench, °C medium immediately below spinnerette..... | 4                  | 30-40                                    | do.....                            | 260-350..... | 300-350.....     | .....                  | .....     |
| Quench air rates in the vicinity of the spinnerette.....    | 5                  | 25                                       | Increases.....                     | 0.1-1.0..... | 0.1-0.5.....     | 4-8.....               | 6-8       |
| Polymer throughput.....                                     | 6                  | 20                                       | Decreases. High <sup>3</sup> ..... | .....        | 4.58.....        | Low <sup>4</sup> ..... | Low.....  |
| Spinnerette orifice capillary:                              |                    |                                          |                                    | s.c.f.m.     | s.c.f.m.         | s.c.f.m.               | s.c.f.m.  |
| Length effects.....                                         | 7                  | 10-15                                    | Increases.....                     | Short.....   | Short.....       | Long.....              | Long..... |
| Length in mils.....                                         |                    |                                          |                                    | 8-80.....    | 8-150.....       | 8-150.....             | 20-150    |
| Length/diameter.....                                        |                    |                                          |                                    | (8).....     | 0.8-3.0.....     | 0.8-2.0.....           | 2-20..... |

<sup>1</sup> On mod.-ratio, percent as compared with \*1.

<sup>2</sup> On left increases effect on mod.-ratio.

<sup>3</sup> 4-8 grams per minute per bifil filament.

<sup>4</sup> 2-6 grams per minute per bifil filament orifice.

<sup>5</sup> Capillary length is proportional to diameter, thus a larger diameter requires a longer length. A better characterization of this is the spinnerette capillary length divided by the spinnerette capillary diameter.

#### EXAMPLE 18

Polycaproamide pellets containing 1.5 percent extractables of 0.1 inch in diameter by 0.1 inch in length were melt spun through a bifilament spinnerette orifice as a type indicated in FIG. 1. The polymer was melted in a  $4\frac{1}{2}$  inch extruder at a temperature of 255 to 265° C. and extruded at the rate of 456 pounds/hour and fed to 8 quench stacks. Each quench stack contained 42 spinnerettes, each spinnerette was subdivided and contained openings for production of 2 bifilament yarn ends on each side of the partition wall. The quench stack contained 168 ends of bifilament yarn and each yarn end was spun at the rate of 0.3 pound/hour/end. Thus, each quench stack produced 57 pounds/hour of 20-denier drawn monofilament yarn.

A peripheral ring of 42 spinnerettes was surrounded with gas maintained at a temperature of 260° C. by two resistance heaters forming a ring on either side of the spinnerette. Each twin orifice had a capillary 10 mils in diameter x 30 mils in length and these twin capillaries were separated from each other by a distance of 2.6 mils.

up roll. Take-up rolls and draw rolls were dual rolls and were canted toward each other  $3^\circ$  to facilitate separation of the wraps. Quartering of the quench stack provided for approximately 10 spinnerettes per quarter. The yarn then passed from the draw roll over a heater 98 inches long at a speed of 4,000 feet/min., thence to false-twist spindles of the type described in U.K. Pat. 931,837 dated July 7, 1963 which combines friction twisting superimposed upon top of the normal rotational speed of 350,000 r.p.m. Two ends were passed through in opposite directions on each twister spindle and threaded up as indicated in the aforesaid patent. The residence time on the 98 inch heater was 0.12 second. The yarn then passed through discharge rolls were the twist was released, said discharge rolls having a peripheral speed of 4,250 feet/min. The yarn was then taken up on a special surface driven winder, which drove 4 sleeves on each of its 4 quarters, each sleeve contained 3 cops and each cop contained 2 ends. Thus, 24 ends were taken up on each of the 4 quarters of the winder. Each sleeve was separately doffable from the winder and each winder took up 96 ends.

The area occupied by the winder was 24 inches on center. Thus, 2 winders accommodated the output of the quench stack.

The r.p.m. of the spindles plus the fractional twist was equivalent to 1.5 million r.p.m. to apply 31 turns/inch at the 4,000 feet/min.

The quality of this false-twisted yarn was somewhat superior to that described in Examples 1 through 14, because of greater uniformity of twist and general freedom from defects which are characteristic of a continuous operation as opposed to a multiple-step operation as described in Examples 1 through 14.

This yarn when knitted into hosiery had essentially the same elastic properties of that described for Example 9, since the elastic properties are the result of the novel filament cross section and the twist turns employed rather than the precise process employed in its manufacture.

Alternately, in place of the false-twist spindles as described in U.K. Pat. 931,837, is the false-twist friction device built by Zimmer Textile Machine Works, Gmbh West Germany and described by Man-Made Textiles and Skinner's Record, September 1967, pp. 110-112. When this this unit is operated at a spindle speed of 20,000 r.p.m., and the friction device is operated at maximum speeds, up to 3,000,000 turns/minute can be imparted to filaments. It is preferred, however, to run the spindles at higher speeds and the friction twist device at lower speeds in order to obtain a more uniform twist.

Since tricot knits have a stitch very similar to the plain knit, e.g., jersey knit stitch, fabric made by tricot knitting exhibits similar elasticity utilizing the bifilament yarns of this invention. Generally, it can be said that tricot fabrics have about 50 to 60 percent less elasticity than jersey knit products. By using bifilament yarns, one can achieve approximately equivalent elasticity in the tricot knit wear as that obtained for jersey knitted round cross section yarns. This represents a substantial improvement in the elasticity for tricot knit wear. These bifilament yarns find utility in women's slacks, swim wear, in leotards and the like, where the characteristics of subtle iridescent sparkle combined with the elastic properties considerably enhance the utility of the textile article made from bifilament yarns. Particularly where sheer fabrics and styling are desirable such as in intimate wear, e.g., night-gowns, housecoats, lounge suits, negligees, peignoirs, and the like, these bifilament yarns have high utility. Tricot knit fabrics and other flat fabrics may be further modified in appearance by employing the processes known as schreiner calendering where the angle and size of the grooving employed tends to increase the contrast thereby resulting in an increase in sparkle. Generally, bright and pastel colors favor the "scintilla look." The acid dyes and fluorescent dyes insure that the sparkle look is emphasized in the finished articles. In mixed fabrics, dark areas decrease the "scintilla look" and bright dyes increase the "scintilla look." Polyamides having amine end groups of 20-30 may be dyed with basic dyes using a pH of 7. Polyamides having amine end groups of 40-50 may be dyed with basic dyes using a pH of 8.

The effect of dyestuff on bifilament textiles in order of decreasing sparkle emphasis is as follows: fluorescent dyes, basic dyes, acid dyes, premetallized dyes and disperse dyes. Other means of increasing the scintilla look are plaiting of the bifilament yarn on the front of dark-colored backing yarn. Also, a considerable increase in the scintilla look can be obtained by doubling the number of bifilament yarns on the face of courses. An opposite effect is obtained if one doubles the number of yarn ends in the wales since this tends to emphasize a flat sheen effect or the "glacé look." By alternating courses used in bifil yarns, the pattern responds to light which tends to highlight reflections obtained which in turn increase the "sparkle effect." With vertical illumination, the hosiery tends to have a glossy appearance which definitely in-

creases the point sparkle. A patterned design generally increases the sparkle.

#### EXAMPLE 19

5 Bifilament yarns produced in accordance with Example 3 except 40 denier monofilament was produced instead of 20 denier monofilament. The 40 denier monofilament had a modification ratio of 2.4. This was placed in tricot knit automotive upholstery having the following yarns: first bar, round cross section nylon, 140 denier/24-filaments bright; second bar, round cross section nylon, 70 denier/12 filaments semidull; third bar, bright filament cross section nylon 40 denier/1 filament. This tricot fabric when bent 90° in daylight, showed a sparkling shimmering sheen where each individual bend of the bifilament yarn appeared as minute point sparkles or "scintillas." The alignment and order of the light reflectance was similar to that shown in hosiery and it is this alignment of the point sparkle which produced a subtle and pleasing shimmer. The sparkle resulted in warmth of fabric appearance without garishness which distinguishes it from prior art novelty sparkle yarns. The tricot fabric had a 5 percent increase in elastic stretch properties compared to a fabric of like construction utilizing a round cross section yarn.

15 It has been found that the high luster and high sheen characteristics of the bifilament yarns of this invention, whether false-twisted or other texturing systems are employed, the reflectivity is relatively unchanged after washing from the original textile article prior to soiling. Therefore, the apparent soiling of such fabrics is largely overcome by a minor reduction in the sheen and the general appearance with respect to soiling is considerably superior to other cross sections such as round, triangular and the like although treated in the similar manner. This property is of particular value in white intimate wear and in pastel colors which would otherwise show considerable soiling in cross sections employed heretofore in the prior art.

20 While the production of the bifilament yarn product of the present invention has been illustrated utilizing separate orifices, those skilled in the art will recognize that other types of orifices may be employed. For example, two holes connected by a thin slot may be used through proper control of spinning conditions which achieve a bifilament as described herein.

25 We claim:

30 1. A method of producing polycaproamide bifilament yarn having improved physical and optical properties for use in ladies' hosiery consisting of extruding molten polycaproamide having a relative formic acid viscosity of about 50 to 65 units at a temperature of from about 255° C. to 270° C. through twin spinnerette orifices, said orifices having a diameter of about 10 mils and a length of about 10 mils and being separated from each other by a distance of about 2 mils and interconnected at the polymer exit surface by a width of not greater than 40 percent of the orifice diameters, the molten polymer entering the spinnerette counterbore at the rate of about 4.78 grams/minute/bifil filament, quenching the polycaproamide yarn at an entering air temperature ranging from about 20° C. to about 41° C. starting at a distance 3 inches below said orifices to a distance of 95 inches below said starting distance at a gas lineal velocity of about 10 lineal feet/minute, fusing the polycaproamide bifilament yarn wherein symmetrically opposed concave sides are formed that intercept at an angle of from 38 to 54 degrees and have a modification ratio between about 1.75 and about 1.95, said method being further characterized in that the polycaproamide bifilament yarn is extruded at a lineal speed of about 1,950 feet per minute, drawn at about 3.98× and subjected to false twisting to a twist level of about 31 turns/inch.

35 2. The method of claim 1 wherein the concave sides of the bifilament yarn intercept at an angle of 46 degrees,

21

3. The method of claim 1 wherein the concave sides of the bifilament yarn intercept at an angle of 49.2 degrees.

22

3,470,686 10/1969 Fleming et al. ----- 57—140  
3,528,128 9/1970 Murakami et al. ----- 18—855

## References Cited

## UNITED STATES PATENTS

|           |         |                 |       |           |
|-----------|---------|-----------------|-------|-----------|
| 2,804,645 | 9/1957  | Wilfong         | ----- | 264—177 F |
| 2,959,839 | 11/1960 | Craig           | ----- | 264—177 F |
| 2,965,925 | 12/1960 | Dietzsch        | ----- | 264—177 F |
| 3,156,085 | 11/1964 | Jamieson        | ----- | 264—177 F |
| 3,308,221 | 3/1967  | Opfell          | ----- | 264—177 F |
| 3,315,021 | 4/1967  | Luzzatto        | ----- | 264—177 F |
| 3,387,327 | 6/1968  | Privott et al.  | ----- | 264—177 F |
| 3,493,459 | 2/1970  | McIntosh et al. | ----- | 264—177 F |
| 3,558,420 | 1/1971  | Opfell          | ----- | 264—177 F |

|   |           |        |               |       |           |
|---|-----------|--------|---------------|-------|-----------|
| 5 | 791,468   | 3/1958 | Great Britain | ----- | 264—177 F |
|   | 816,877   | 7/1959 | Great Britain | ----- | 264—177 F |
|   | 1,112,938 | 5/1968 | Great Britain | ----- | 264—177 F |
|   | 1,023     | 2/1963 | Japan         | ----- | 264—177 F |
|   | 9,535     | 5/1965 | Japan         | ----- | 264—177 F |

10 JAY H. WOO, Primary Examiner  
U.S. CL. X.R.  
161—177; 264—210 F; 425—464

## FOREIGN PATENTS

UNITED STATES PATENT OFFICE  
CERTIFICATE OF CORRECTION

Patent No. 3,737,505

Dated June 5, 1973

Inventor(s) Garland L. Turner et al.

It is certified that error appears in the above-identified patent  
and that said Letters Patent are hereby corrected as shown below:

Column 1, line 20, "preefrably" should be --preferably--.

Column 3, line 28, "warps" should be --wraps--.

Column 4, line 36, "elastically" should be --elasticity--.

Column 4, line 53, "yarns" should be --yarn--.

Column 5, line 48, "lost" should be --lose--.

Column 6, line 1, "filament" should be --bifilament--.

Column 6, line 2, "significant" should be  
--significantly--.

Column 8, line 2, "trifiament" should be --trifilament--.

Column 10, line 19, "wrap" should be --warp--.

Table 2, under "Percent Work of Recovery", Example  
No. 3, "4.4" should be --44.4--.

Table 2, under "Ankle Elongation, %, 15, Example  
13, "6" should be --86--.

Signed and sealed this 8th day of January 1974.

(SEAL)  
Attest:

EDWARD M.FLETCHER, JR.  
Attesting Officer

RENE D. TEGTMEYER  
Acting Commissioner of Patents